

## UNITED STATES PATENT OFFICE

CHARLES F. GOLDTHWAIT, OF MOUNT LEBANON TOWNSHIP, ALLEGHENY COUNTY, PENNSYLVANIA, ASSIGNOR, BY MESNE ASSIGNMENTS, TO TEXTILE MACHINERY CORPORATION, A CORPORATION OF DELAWARE

## MODIFIED COTTON

No Drawing.

Application filed June 4, 1931. Serial No. 542,105.

This invention relates to a new cellulose fibre made from cotton, or alternatively, to a cotton fibre with a greatly modified structure.

5 This application is akin to my co-pending application, Serial No. 476,441, filed August 19, 1930, (now abandoned) and to two other applications Serial Nos. 542,106 and 502,107 filed on even date herewith, for process of 10 strengthening cellulose.

An object of this invention is to provide a modified cotton fibre which, by change of structure, becomes a new cellulose fibre.

15 A further object of the invention is to produce a modified cotton fibre whose strength is far greater than that of the natural or otherwise modified cotton.

20 The value of this fibre lies in its great strength, which is far superior to that of other known cottons or modified cottons. The processes employed consist in the treatment of cellulose, particularly cotton, with swelling agents such as caustic soda, under 25 conditions such as hereinafter specified.

25 This treatment may be followed by heating the cotton in a soap or other solution to enhance the strengthening effect.

The novelty of this invention is proved by 30 X-ray analysis, the new fibre giving an X-ray diffraction diagram that is different from that of any other known cotton or modified cotton.

35 The new fibre is made from natural cotton conveniently described in the form of yarn, but this is intended to embrace the use of cotton in other forms, such as loose fibre or cloth.

40 The new fibres are very different in outward appearance from natural cotton fibres, but retain approximately the same dimensions.

45 They resemble, in appearance, other modified cottons, particularly those produced by ordinary mercerization, but they are fundamentally different in structure within the individual fibres from natural, mercerized or other known modified cottons.

50 There are numerous grades of cotton, and so far as known, they can all be converted to the new type of fibre. Comparable results

to those of ordinary American cottons have also been obtained with Egyptian cotton.

The result, in terms of strength, will necessarily vary with the kind of cotton used, and the construction, if for example, it is in 55 the form of yarn.

The new material can be made in a great variety of strengths from that of mercerized cotton on up, some samples running as high as twice the original cotton strength when 60 tested in a dry atmosphere.

Therefore, it is not intended to limit this application to cotton of any specific gain in strength.

65 It has been found by various investigators, by means of X-rays, that the natural forms of cellulose have characteristic internal forms of structure. The present knowledge of the subject indicates that all cellulose consists very largely, if not entirely, of elongated particles called "micelles". These particles have a very definite type of structure, which is commonly described as crystalline.

70 In some fibres, particularly in natural cotton, the micelles are arranged in irregular spiral forms around the fibre axis, an arrangement which is not conducive to the greatest strength of cellulose.

75 In other celluloses, such as ramie, the micelles have grown naturally in the plant in quite perfect parallel arrangements, and such fibres are usually very strong.

80 The natural plant fibres each have characteristic sizes, shapes and other physical properties which are peculiar to them, as well as the form of internal structure.

Treatment of these natural fibres with chemicals, notably the mercerization of cotton, may change the external appearance and otherwise alter the character of fibres to some extent. But as far as known, such treatments have not greatly influenced the internal structural arrangements of the individual fibres.

85 From the X-ray studies, it has been found that there is a close connection between the 90 strength of the cellulose of a fibre and the degree of parallelism of its micelles. In general, the higher the degree of parallel orientation, the higher is the strength, but particularly when the comparison is made within 100

a class. That is to say, cotton with cotton, viscose rayon with viscose rayon, cuprammonium rayon with cuprammonium rayon.

This has been particularly well exemplified by Professor George L. Clark, of the Department of Chemistry, University of Illinois, in a paper appearing in "Industrial and Engineering Chemistry", May, 1930, volume 22, page 474 et seq. and considering especially cellulose in other forms than cotton.

This article deals at length with the orientation of the micelles in cellulose, and Figure 8 in said paper is illuminative.

For example, certain strands of rayon of inferior strength show a higher random arrangement of the micelles, while others made from the same materials, but with greater stretching and tensioning, show the micelles much more nearly parallel, and have much higher strengths. (See Figures 16, 17, 18, 19 and 20 of the above article).

And while these materials are outwardly similar in form, they are really different materials with different properties, owing to their different internal structures.

The new fibre forming the subject-matter of this invention has a similar X-ray diagram to that of the strongest rayons, indicating a similarity in internal structure, but it differs from rayon in that it has never been through a state of dispersion in a liquid as in rayon manufacture. It has instead been converted directly from natural cotton by suitable manipulation and treatment in the fibrous form with chemicals.

It is, of course, to be understood that parallelism of micelles is not the only important factor in the strength of cellulose. Its strength depends fundamentally upon the attraction for each other of the atoms, molecules and other particles of which the substance is composed.

According to the present state of knowledge, it is supposed that the more perfect parallel arrangement of micelles causes a closer packing of these structural units and promotes the attraction between them.

The extra strength is, therefore, partly due to the closer association of the micelles or to the development of new points of attraction between them.

The novel nature of the new fibres is shown by both the increased strength and the X-ray diagram, which indicates the new structural form.

In order to illustrate and define the character of this new fibre, X-ray analyses were made, covering untreated natural cotton, commercial mercerized yarn, and yarn treated in accordance with the present invention.

For the sake of examples, in natural Egyptian cotton the double strand strength of 60/2 yarn measured 1.53 pounds in a dry atmosphere but 1.75 with standard humidity

conditions, and the X-ray diffraction diagram of its fibres showed the usual random arrangement of micelles for natural cotton. The same yarn, after being commercially mercerized, measured 2.07 pounds and its fibres shows a slightly improved diagram with a slightly greater degree of parallel arrangement of micelles. But when treated according to the teachings of my applications above referred to, the yarn measured 2.54 pounds and showed the X-ray diagram of highly oriented cellulose. These tests were conducted in the ordinary laboratory dry atmosphere, except as stated.

These figures are taken from accurate tests made in the laboratories of the Mellon Institute of Industrial Research, University of Pittsburgh.

As an instance where cotton yarn was increased to approximately double strength when tested in an ordinary dry atmosphere, the following procedure was used: Two-ply cotton of the construction commonly known as mercerizing-twist was immersed in dry skeins (without previous boiling-out) in a 35% solution of caustic soda containing a suitable amount of wetting agent for use in caustic soda solution.

It was allowed to shrink freely in this solution. After a thorough soaking the yarn was squeezed and put on rollers in a frame while still containing the caustic. It was then stretched to approximately its original length, and further stretched while washing with cold water to approximately 4% beyond its original length.

The yarn was neutralized with acid while in the stretched condition, washed in the loose form, stretched again, and dried as usual with heat. While still in the stretched condition it was boiled for fifteen minutes in a 2% solution of soap, then washed and dried while still held taut.

"Retaining approximately its original dimensions" means that the fibres in a given yarn appear in the modified form at practically the original length; that the shapes and dimensions of the cross section are somewhat changed; but that there is no appreciable amount more or less fibre substance in a cross section. Superficially the fibres would appear to be of the same size as before treatment.

This invention is not limited to cotton prepared with caustic soda but may include that prepared by other alkalies or swelling agents for cellulose; it may also include modified cotton of the character specified, produced by heating in other colloidal solutions than soap, particularly so-called wetting agents and some salts of organic acids, including organic salts or soaps such as those made with the ethanolamines and other organic bases.

Experiments and tests have proved that there is a sufficient conversion of fibres to im-

part an unusual strength to yarns and to cause them to show the typical diagram for highly oriented micelles when suitably analyzed by X-rays. These effects can be taken as proof 5 that the cotton has been very completely converted to a new and more valuable fibrous material.

Throughout this application and claims where the word "oriented" or the like is used, 10 it will be understood that the sense of the word must be construed as meaning "an arrangement parallel with the fibre axis."

In the article above referred to as appearing in the "Industrial And Engineering 15 Chemistry", Figure 13 shows an X-ray diffraction diagram of ordinary cotton, while Figure 2 therein shows an X-ray diffraction diagram of native ramie having a high degree of orientation of micelles parallel to 20 the fibre axis. The new article of manufacture claimed herein, namely a modified cotton fibre of high strength, may be produced from ordinary cotton and has given an X-ray diffraction diagram practically identical with 25 the ramie diagram shown in Figure 2, of that article.

Of course, the specific structures mentioned herein are not to be taken as limiting this invention in any way, and it is to be understood 30 that various modifications and changes in the method of treatment may be employed without departing from the invention herein set forth and hereafter claimed.

The invention is hereby claimed as follows:

- 35 1. A modified cotton fibre retaining approximately its original dimensions and characterized by the X-ray diffraction diagram of highly oriented cellulose.
- 40 2. A new article of manufacture comprising a modified cotton fibre having its micelles approximating perfect orientation and having a tensile strength far greater than that of the natural or otherwise modified cotton.
- 45 3. A modified mercerized cotton fibre retaining approximately its original dimensions and characterized by the X-ray diffraction diagram of highly oriented cellulose.
- 50 4. A new article of manufacture comprising a modified mercerized cotton fibre having its micelles approximating perfect orientation and having a tensile strength far greater than that of the original mercerized cotton.

In testimony whereof I have signed my 55 name to this specification.

CHARLES F. GOLDTHWAIT.